

[54] **COLOR REVERSAL PROCESS AND DEVELOPER**

[75] Inventor: **Robert P. Molenda, St. Paul, Minn.**

[73] Assignee: **Minnesota Mining and Manufacturing Company, St. Paul, Minn.**

[22] Filed: **Aug. 14, 1972**

[21] Appl. No.: **280,263**

**Related U.S. Application Data**

[63] Continuation-in-part of Ser. No. 188,616, Oct. 12, 1971.

[52] **U.S. Cl.** ..... **96/59; 96/22; 96/55;**  
96/66 R

[51] **Int. Cl.** ..... **G03c 5/50; G03c 5/30**

[58] **Field of Search**..... 96/22, 59, 66 R, 55

[56] **References Cited**

**UNITED STATES PATENTS**

3,165,407 1/1965 McCarthy ..... 96/22

|           |         |                   |         |
|-----------|---------|-------------------|---------|
| 3,295,975 | 1/1967  | Meckl .....       | 96/59   |
| 3,300,305 | 1/1967  | Pesch et al. .... | 96/22   |
| 3,335,004 | 8/1967  | Wrisley .....     | 96/22   |
| 3,615,509 | 10/1971 | Klein .....       | 96/66 R |
| 3,615,522 | 10/1971 | Ohi .....         | 96/66 R |
| 3,658,525 | 4/1972  | Bent .....        | 96/66 R |

*Primary Examiner*—Mary F. Kelley

*Attorney, Agent, or Firm*—Alexander, Sell, Steldt & Delahunt

[57] **ABSTRACT**

Rapid access positive color development of a silver halide photographic element is achieved by developing the element in a monobath which includes a photographic color developing agent, a black and white photographic developer, and a dye-formation inhibitor, to develop a black and white image. The element is thereafter treated to reduce the inhibiting action of the dye-formation inhibitor to permit formation of a colored, positive image.

**32 Claims, No Drawings**

## COLOR REVERSAL PROCESS AND DEVELOPER

This application is a continuation-in-part of U.S. application Ser. No. 188,616, filed Oct. 12, 1971.

The present invention relates to photographic color development technology, and more particularly relates to a color reversal monobath and a process for its use, and to photographic kits adapted to prepare such monobaths.

A widely used process for reversal color development of silver halide photographic films employs a succession of baths through which exposed photographic films must be passed. For example, a first bath may include a black and white developing agent which reduces silver halide in latent image areas of a film to silver, forming negative silver image therein. Thereafter the film may be uniformly exposed to light to form fog centers in undeveloped areas of the film, and then treated with a color developer solution in which a color developing agent reduces silver halide in the fogged areas to silver, and is itself oxidized. The oxidation product of the developer reacts with one or more color couplers which may be distributed throughout various layers of the film to form dyes therein. The silver images may then be bleached from the film, and unreacted silver halide may be removed therefrom by "fixing" to thus provide positive, colored images. To avoid cross-contamination of the various processing baths, a number of intermediate wash baths are commonly employed. Further, a "stop" bath is ordinarily utilized to halt black and white development immediately after treatment of the film in the black and white developer bath.

As will be evident from the above description, the process described employs many steps and utilizes many different processing baths. In addition, the shelf-life of these prepared solutions are poor. Further, the above procedure must be very carefully regulated in order to provide satisfactory photographic color reproductions. Moreover, the time which is required to fully process an exposed roll of color film (a major cost factor) is inordinately long. A faster, more efficient, less-detailed positive color development process is hence much to be desired.

It is an object of the present invention to provide a color developer monobath for rapid, positive color processing of a photographic element.

It is another object of the invention to provide a color reversal development process by which color photographic elements may be rapidly developed.

It is yet another object of the invention to provide a photographic color development kit from which the monobaths of the invention may be prepared.

Briefly, the present invention in one embodiment relates to a photographic color reversal development process which comprises:

A. treating a photographic element having a hydrophilic colloid (e.g., gelatin) silver halide layer bearing a latent image with an aqueous monobath which includes

1. at least one photographic color developing agent, capable, upon oxidation thereof, of reacting with a photographic color coupler to form a dye;
2. at least one black and white developing agent having a polarographic half-wave potential at pH

10.0 or from about -10 millivolts to about -187 millivolts, and

3. a water-soluble dye-formation inhibitor which is capable of preventing said color developing agent from coupling with a color coupler, thereby to imbibe the silver halide layer with the monobath and to develop solely a negative black and white silver image therein;
- B. thereafter fogging the silver halide layer so as to render the layer developable in non-imaged areas;
- C. without intermediate removal of the imbibed monobath, treating the layer to reduce the inhibiting effect of said dye-formation inhibitor, and
- D. allowing development of a positive color image therein in the presence of a color coupler.

The practice of this invention includes the use of either photographic elements which contain couplers originally distributed in at least one emulsion layer or elements which contain spectrally sensitized silver halide and require the subsequent addition of color couplers as by a later bath solution.

Black and white and subsequent color development in the process of the present invention is believed to occur as follows:

25 Upon treatment of a silver halide photographic element bearing a latent image with the aqueous monobath described above, silver halide in latent image areas is reduced by the black and white developer to form a silver image. Because of the presence of the water-soluble dye-formation inhibitor, substantially no dye formation occurs at this time. Any of the color developer which has reduced silver halide (and which in turn has been oxidized) reacts with the dye-formation inhibitor (e.g., sulfite) to form a stable reaction product (e.g., a monosulfonate derivative). Dye formation during black and white development of the latent image is thus prevented. After black and white development of the latent image has been completed (so that substantially no reducible silver halide remains in latent image areas), the element is removed from the developer bath and is "fogged," e.g., by exposure thereof to light, or by treatment thereof with known chemical fogants such as hydrazine, potassium borohydride, amine boranes, etc. At this point, the element still retains imbibed therein the monobath. Upon subsequent treatment of the element so as to reduce or eliminate the inhibiting effect of the dye-formation inhibitor in the imbibed monobath, color development of the element by the imbibed color developing agent may occur in those areas of the element which were fogged after black and white developing forming a positive colored image when color couplers are present.

The inhibiting effect of the dye-formation inhibitor may be reduced, for example, by treating the element with a composition which, for example, neutralizes or reduces the tendency of the inhibitor to form a reaction product with oxidized color developer. For example, when sulfite is employed as a dye formation inhibitor, the element may be treated with a solution of a sulfite-reactive composition to neutralize sulfite in the imbibed monobath. The inhibiting effect of the dye formation inhibitor may be reduced, in a preferred embodiment, by decreasing the concentration of inhibitor in the imbibed layer, as by washing the imbibed layer with a solution which is capable of dissolving the inhibitor. Aqueous solutions of from about pH 7 to about pH 13 (most preferably above pH 10) are preferred for this

procedure, particularly when sulfite is employed as the dye-formation inhibitor. Such solutions preferably include a basic ingredient such as sodium hydroxide, sodium carbonate, trisodium phosphate dodecahydrate, etc., to render the solution alkaline, and may further include such photographic additives as sodium sulfite, fogging agents, surfactants, color couplers (particularly when a coupler-free photographic element is to be developed to form a monochromatic image), etc. When sulfite is employed as the dye-formation inhibitor, then the washing solution is preferably chosen so as to be sulfite-dissolving; i.e., it exhibits the capacity to remove sulfite from the imbibed monobath solution to thus permit color development to occur. When the inhibiting effect is accomplished for example by forming an amine salt, the pH of the wash bath should be high enough to convert the salt to an amine. Although the solution preferably includes such additives as are exemplified above, satisfactory results have been obtained by simply washing the fogged element with water.

The dye-formation inhibitors of this invention may operate by selective reaction with oxidized color developer to prevent them from coupling to form a colored dye. The inhibitors may also act upon the developing agent to prevent its oxidation so that no colored dye is formed. For example, this latter inhibiting mechanism may be performed by blocking the amine group(s) on the color developing agents in the bath. The blocking may be accomplished, for example, by forming amine salts of the color developing agents (e.g.,  $-\text{NH}_3^+\text{Cl}^-$ ,  $-\text{NH}_2\text{CH}_3^+\text{Br}^-$ ,  $-\text{NH}(\text{CH}_3)_2^+\text{OH}^-$ ). The particular conditions and parameters of the monobath solution depend to some degree upon the particular mechanism which is selected to inhibit the formation of dye by the coupling of developing agent and color coupler.

Where the dye formation inhibitor is selected so as to form with the oxidation product of the color developing agent a reaction product which is either colorless or removable, the following characteristics in the monobath are generally preferred:

- A. The monobath should have a pH of about 8.5-14 (most preferably about pH 10.0-11.0);
- B. The dye-formation inhibitor should be present in sufficient quantity so that substantially all dye formation in a silver halide photographic element is restrained in said monobath after exposure of said element therein to light.

Where the dye formation inhibitor acts by blocking the reactive amine group(s) of the color developing agent it may be desirable to have the pH of the bath below 8.5 and in many instances well below 7.0 (as low as 3.0).

With either mechanism, however, the developing agents must still possess half-wave potentials within the limits prescribed previously and hereinafter.

As used herein, "photographic color developing agent" refers to a compound capable of reducing silver halide to silver and in turn being oxidized, the oxidation product thereof being reactive with a photographic color coupler to form a dye. Photographic color developing agents of the p-phenylenediamine type (e.g., 2-methyl-4-[N-ethyl-N-( $\beta$ -methylsulfonamidoethyl)-amino] aniline and 4-amino-N-ethyl-N-( $\beta$ -hydroxyethyl)-aniline and their salts, are preferred. Such color developing agents are known to the art, and reference is made to Mees and James, Eds, *The Theory of the Photographic Process*, 3rd Ed., MacMillan, New York,

1966, Chapter 17. Color developing agents having a polarographic half-wave potential at pH 11.0 of from about -159 millivolts to about -305 millivolts are particularly preferred.

5 By "black and white photographic developer" employed herein, reference is made to one or more black and white developing agents which are capable of reducing silver halide to silver but which are incapable of reacting, in oxidized form, with a photographic color 10 coupler to form a dye; this term includes mixtures of black and white developing agents, for example, hydroquinone and 1-phenyl-3-pyrazolidinone. Such developing agents include those known to the art such as those of the hydroquinone series (e.g., hydroquinone, chloro-15 hydroquinone, bromohydroquinone, methylhydroquinone, dichlorohydroquinone, o-methoxyhydroquinone and catechol), those of the p-aminophenol series (e.g., N-methyl-p-aminophenol sulfate, p-hydroxyphenylglycin and p-aminophenol) and those of the pyrazolidinone series, particularly 3-pyrazolidinones such as 20 1-phenyl-3-pyrazolidinone. The black and white developing agents of the invention as defined above preferably are further characterized by the formula

25

Y—M—X

wherein M is a cyclic organic nucleus (e.g., benzene, pyrazolidinone) which includes no cyclic atoms other than carbon and nitrogen, Y is an OH group bonded to a cyclic carbon atom of said nucleus, and X is a hydrogen atom or a hydroxyl, alkylamino, carboxyalkylamino, amino, alkyl or aryl group, X being bonded to a cyclic atom of said nucleus. The black and white photographic developer of the invention includes at least one black and white developing agent having a polarographic half wave potential at pH 10.0 of from about -10 millivolts to about -187 millivolts.

The use of half-wave potentials ( $E^{1/2}$ ) for describing the useful developing agents, both color and black and white, is an efficient and meaningful way of characterizing the invention. Thermodynamically, the half-wave potential can be related to the reaction rate of the developing agents with silver halide. The greater the free energy of the reaction process, (here, the greater the tendency of the developing agent to release electrons), the more positive is its oxidation half-wave potential according to the Lewis and Randall Convention. Reference is made to Bent et al., *Chemical Constitution, Electrochemical, Photographic and Allergenic Properties of p-Amino-N-dialkylanilines*, J. Am. Chem. Soc., 73, 3100, 1951; Willis et al., *The Relative Importance of Adsorption and Electrode Potential in Determining the Rate of the Induction Process During Photographic Development. II. Hydroquinones*, Photographic Science and Engineering, Vol. 14, No. 2, pages 149-152 (1970); and Willis et al., *The Relative Importance of Adsorption and Electrode Potential in Determining the Rate of the Induction Process During Photographic Development. I. The p-Aminophenols and p-Phenylenediamines*, Photographic Science and Engineering, Vol. 14, No. 2, pages 141-148 (1970).

65 The Lewis and Randall Convention (G. N. Lewis and N. Randall, *Thermodynamics*, McGraw Hill, New York, 1923, page 389) has been employed herein with respect to the values of "polarographic half wave potential" of black and white and color photographic developing agents. The polarographic half wave potentials

referred to herein are oxidation potentials which may be experimentally determined by employing the method reported in Julian and Ruby, *The Use of Stationary Platinum Microelectrode in the Determination of Half Wave Potentials*, J. Am. Chem. Soc., 72, 4719, 1950, the values being taken relative to the hydrogen electrode at pH 10.0 (black and white developing agents) or pH 11.0 (color developing agents). The concentration of black and white developer in monobaths of the invention may be very low (e.g., at least as low as 0.0045 moles/liter).

The particular controls used on a system depend, of course, upon the particular materials used. Since the basic desired mechanism of the process is to have the black and white developer favorably compete with the color developer for the image silver halide certain considerations must be given in the formulation of the monobath compositions. Where the black and white developer has a significantly higher half-wave potential than the color developer, there is already a strong tendency for the black and white developer to develop the image and a relatively weak color dye formation inhibitor (either by selection of material or low concentration) may be used. When there is not a substantial dif-

ference between the half-wave oxidation potentials of the two agents additional control must be effected over the monobath to insure the preferential development by the black and white agent. This may be done by increasing the strength of the dye-formation inhibitor (by selection of material or increasing the concentration of such) and/or increasing the tendency of the black and white agent to develop the image by increasing the concentration of that agent. In general, however, the parameters of half-wave potentials used in describing the useful developing agents define the limits of useful materials for each category of developing agents. That means, for example, that a black and white developer with a half-wave potential at pH 10 of less than -187 millivolts will not produce satisfactory results in this process even by exercising the known controls over the reaction mechanisms. The process can be performed with substantially all developing agents selected from within the half-wave potential ranges for each of the agents. The half-wave potential therefore satisfactorily generically describes the materials which can be used in this process.

A listing of some known developing agents and their half-wave potentials follows:

25

TABLE OF SOME OXIDATION POLAROGRAPHIC HALF-WAVE POTENTIALS

| COLOR DEVELOPERS | pH of Measurement |        |        |                                                                 |
|------------------|-------------------|--------|--------|-----------------------------------------------------------------|
|                  | 9.2               | 10.0   | 11.0   |                                                                 |
| <u>Compound</u>  |                   |        |        |                                                                 |
|                  | -279.5            | -266.0 | -222.0 | N,N-diethyl-p-phenylenediamine                                  |
|                  | -321.5            | -229.0 | -190.0 | 2-amino-5-diethylaminotoluene (CD-2)                            |
|                  | -269.5            | -247.0 | -190.0 | 4-amino-N-ethyl-N-(p-methanesulfonamidoethyl)m-toluidine (CD-3) |
|                  |                   | -188.0 |        | 4-amino-2-methyl-N-ethyl-N-(p-hydroxyethyl)aniline (CD-4)       |

TABLE OF SOME OXIDATION POLAROGRAPHIC HALF-WAVE POTENTIALS (CONTINUED)

| BLACK & WHITE DEVELOPERS | pH of Measurement |                        |                             |      |        |      |                                            |
|--------------------------|-------------------|------------------------|-----------------------------|------|--------|------|--------------------------------------------|
|                          | 8.0               | 9.0                    | 10.0                        | 10.7 | 11.0   | 12.5 |                                            |
| <u>Compound</u>          |                   |                        |                             |      |        |      |                                            |
|                          | -256.0            | -181.0                 | -152.0                      |      |        |      | chlorohydroquinone                         |
|                          | -181.0            | -126.0                 | -29.0                       |      |        |      | methylhydroquinone                         |
|                          | -206.0            | -166.0                 | -129.0                      |      |        |      | hydroquinone                               |
|                          | -215.0            |                        | -141.0                      |      |        |      | phenidone                                  |
|                          |                   | -246.0                 | -188.0 (borderline utility) |      |        |      | hydroquinone monosulfonate                 |
|                          |                   | (outside useful range) | -191.5                      |      | -151.5 |      | hydroquinone monocarboxylic acid hydrazide |

This table simply illustrates that these black and white developers are more reactive than these color developers, using the oxidation half-wave potentials as an index of their reactivity. The more positive the number, the more reactive is the particular developer, at any given pH. The change in half-wave potential with pH is expected, and indicates that the developers (any developer) become more reactive as the pH is increased. The lesser reactive black and white developers, phenidone and hydroquinone monosulfonate are noteworthy because these developers are not reactive enough to scavenge silver halide before the color developer present can react to form a dye image. Developers (black and white developers) which are more reactive than these representative developers (that is more reactive than phenidone and hydroquinone monosulfonate) are found to give excellent positive images when used in the manner described in our invention.

Good results are obtained when the color developing agent contributes at least 40 percent up to about 95 mole percent of the total moles of developer (black and white plus color developing agents).

It is further desired that the monobaths of the invention include at least 0.02 moles/liter up to the solubility limit of color developing agent in the monobaths. Preferably, from about 0.06 to 0.10 moles of color developing agent per liter is employed.

The water-soluble, dye-formation inhibitor which is preferably employed in the present invention is a composition, such as sulfite, which is capable of reacting with oxidized color developer which may be formed during the black and white development step to form therewith a stable reaction product. Sulfite is preferred. By "sulfite" as used herein, reference is made to sulfite and bisulfite compounds which, when dissolved in water, liberate sulfite ion. Preferred sources of sulfite ion include ammonium sulfite and the alkali metal sulfites such as sodium sulfite, potassium sulfite, etc., particularly sodium sulfite. The monobath of the invention must contain sufficient dye-formation inhibitor to restrain substantially all dye formation in the silver halide photographic element in the monobath after exposure of the element in the monobath to light. In its preferred embodiment, the monobath of the invention employs inhibitor (e.g., sulfite) in a concentration of 0.10 moles/liter and more preferably from about 0.15 to about 0.48 moles/liter. For purposes of permitting rapid color development to occur, it is preferred that the mole ratio of sulfite/color developer be at least 0.97 and more preferably 1.46 to 7.8. Other suitable dye-formation inhibitors which form reactive products with oxidized color developing agents include ascorbic acid, citrazinic acid, 4-hydroxy-3-butanone, etc.

Other such dye-formation inhibitors include hydroquinone monocarboxylic acid hydrazine. Dye-formation inhibitors of this type which form reaction products with oxidized color developing agents and which are useful in the invention may be selected by reference to the following simple test:

To 50 milliliters of an aqueous test solution containing 0.3 grams of 2-methyl-4-diethylamino aniline hydrochloride, 0.05 grams of 1-hydroxy-N-[ $\beta$ -(2-acetamidophenyl)-ethyl]-2-naphthamide and 2.0 grams of sodium carbonate are added 0.006 moles of a candidate dye-formation inhibitor. To the resulting solution, after mixing, is added 2 drops of an aqueous solution containing, per liter, 75 grams of potassium

ferricyanide. Absence of the development of color in the solution upon addition of the ferricyanide solution indicates that the candidate compound is a dye-formation inhibitor of the invention.

Those materials known in the photographic industry as competing couplers or colorless couplers suitably act as dye-formation inhibitors in the practice of this invention. For example, U.S. Pat. No. 2,742,832 lists a number of competing couplers which would be suitable as inhibitors which form reaction products with oxidized color developing agents in this invention.

Dye-formation inhibitors which act to prevent oxidation of the color developer may be chosen according to the following test:

Any compound which when added to the monobath system reversibly reduces the oxidation potential of the color developer below that of silver is effective as an inhibitor which prevents oxidation of the color developing agent. This may readily be measured by known electrolytic cell techniques. By reversible it is meant that some alteration of condition in the bath or subsequently added material can regenerate the color developing agent from the blocked color developing agent.

It is within the scope of this invention to block the color developing agent prior to its addition to the black and white developer. That is, it is within the scope of the invention to add the color developing agent and dye-formation inhibitor as one compound, for example, by adding the color developing agent in its already inhibited form. This form may be for example a blocked amine salt or a complex of the color developing agent.

The monobaths of the invention may, of course, include various other photographic adjuvants such as bromide ion, surfactants, color couplers, benzyl alcohol, ethylene glycol, thiocyanates and the like.

After development of the colored, positive image, the ordinary process steps normally used in finishing the picture should be used here. That is, after the bath to remove the inhibiting effect, there should be an acid stop bath, then bleach bath, fix bath (or bleach/fix bath), wash, and stabilizing bath. Hardeners may be added to any or all of the stop, bleach, fix or bleach/fix baths, or a prehardening bath may be used prior to development in the monobath. The compositions of such baths are well known in the art and need not be discussed here.

Between the development bath and the bath to remove the inhibitor a quick wash step has been found desirable to remove the solution retained on the surface of the photographic element so as to prevent contamination of the latter bath. This wash is not of sufficient length of intensity as to reduce the inhibiting effect, but is only used to remove the solution held by surface tension on the photographic element. Of course if one is using water as the inhibitor removing second bath such a quick wash would be unnecessary.

Although the photographic color developer monobaths of the invention are surprisingly stable over extended time periods in solution form, it may be desirable from a commercial standpoint to provide color developer kits from which the monobaths of the invention may be prepared. Accordingly, in another embodiment the present invention relates to a color developer kit from which can be prepared positive-acting color development monobaths for color development of silver halide photographic elements. The kit comprises a plurality of packages containing predetermined quantities

- of developer monobath ingredients, the kit including
- A. at least one photographic color developing agent capable, upon oxidation thereof, of reacting with a photographic color coupler to form a dye,
  - B. at least one black and white developing agent having a polarographic half-wave potential at pH 10.0 of from about -10 millivolts and about -187 millivolts; and
  - C. sulfite in sufficient quantity to provide a sulfite/-color developer mole ratio of at least 0.97 (and preferably 1.46 to about 7.8).

In a two-package kit, for example, one package may contain an acidic solid or aqueous liquid which includes sulfite, color developing agent and black and white developer, and the second package may contain an alkaline concentrated liquid or solid which includes an alkaline substance such as sodium hydroxide, a source of bromide ion and sulfite. A three-package kit may have a first package which includes a concentrated, acidic solid or aqueous liquid containing a color developing agent plus sulfite, a second package which includes a concentrated acidic solid or aqueous liquid which contains the black and white photographic developer plus sulfite, and a third package containing a concentrated alkaline solid or aqueous liquid which includes a base such as sodium hydroxide, a source of bromide ion, and sulfite. For reasons of economy, it is desired that each package be made as concentrated as practicable. Although it is desired that the contents of each package be in solution form, it may be desirable in some instances to provide certain of the package contents in the form of aqueous dispersions, thereby enabling high concentrations of ingredients to be achieved and further promoting easy dissolution of the dispersed ingredients when the working monobath is prepared. It may be desirable to some instances to provide the monobath ingredients in solid, preferably powdered form. The contents of each package of the kits of the present invention are carefully premeasured so that the monobaths of the invention may be prepared by adding the entire contents of each package sequentially to water, and diluting to a predetermined volume. Thus, sufficient basic material (e.g., sodium hydroxide) must be included within the kit to provide the resulting monobath with a pH of from 8.5-14, sufficient dye formation-inhibitor must be provided so that the resulting monobath does not permit dye formation to occur during black and white development therein of a photographic element, etc. In preparing monobaths of the invention, e.g., from developer kits, color developing agent solubility problems are largely avoided by first forming an aqueous solution of color developing agent, and thereafter adding the alkaline ingredients thereto.

In the practice of this invention, when it is stated that there is substantially no dye formation, it is meant that no colored form of a dye which cannot be removed from the photographic element is formed. The formation of colorless dyes or intermediates or readily removable (e.g., water soluble) dyes is not the type of dye formation which must be restrained in the practice of this invention.

The invention may be more readily understood by reference to the following illustrative, non-limiting examples:

#### EXAMPLE 1

A gelatino silver halide photographic film containing

red, green, and blue-sensitive layers (the layers containing appropriate color couplers dispersed therein by a solvent dispersion technique) was exposed through a grey wedge (continuous, logarithmic density wedge) in a sensitometer and was developed for 3 minutes at 70°F. in total darkness in a monobath of the following composition:

|    |                              |      |     |
|----|------------------------------|------|-----|
| 10 | Water                        | 800  | ml. |
|    | Sodium hexametaphosphate     | 2.0  | g.  |
|    | 2-methyl-4-diethylamino      |      |     |
|    | aniline (color developer)    | 12.0 | g.  |
|    | Sodium sulfite               | 50   | g.  |
|    | Hydroquinone                 | 6 g. |     |
|    | Sodium carbonate (anhydrous) | 40   | g.  |
|    | Potassium bromide            | 2.0  | g.  |
|    | Water to                     | 1000 | ml. |

Thereafter, the film carrying imbibed monobath was 20 placed in an aqueous solution containing 40 g. per liter of sodium carbonate, and was exposed therein to light for 3 minutes. The film was then washed with water, bleached for 2 minutes in a bleaching bath consisting of

|    |                            |      |     |
|----|----------------------------|------|-----|
| 25 | Water                      | 900  | ml. |
|    | Potassium ferricyanide     | 75   | g.  |
|    | Potassium bromide          | 15   | g.  |
|    | Glacial acetic acid        | 10.0 | ml. |
|    | Sodium acetate             | 5.0  | g.  |
| 30 | Potassium aluminum sulfate | 15.0 | g.  |
|    | Water to                   | 1000 | ml. |

was washed again, and then treated for 2 minutes with a conventional fixing solution of the following composition:

|    |                            |      |     |
|----|----------------------------|------|-----|
| 35 | Water                      | 500  | ml. |
|    | Sodium thiosulfate         | 240  | g.  |
|    | Sodium sulfite             | 15.0 | g.  |
|    | Glacial acetic acid        | 48.0 | ml. |
|    | Boric acid                 | 75.0 | g.  |
|    | Potassium aluminum sulfate | 15.0 | g.  |
|    | Water to                   | 1000 | ml. |

40 After washing and drying, the film bearing a positive color image exhibited the following densitometric properties:

| 50 |                                  | D <sub>min</sub> | D <sub>max</sub> |
|----|----------------------------------|------------------|------------------|
|    | to Blue light (yellow density)   | 0.58             | 2.93             |
|    | to Green light (magenta density) | 1.62             | 3.16             |
|    | to Red light (cyan density)      | 0.92             | 3.42             |

#### EXAMPLE 2

Example 1 was repeated exactly except that the aqueous sodium carbonate solution was replaced with 60 distilled water. Similar results were obtained.

#### EXAMPLE 3

A silver halide photographic element similar to that 65 employed in Example 1 was exposed through a grey wedge to light and then developed for 5 minutes at 70°F in total darkness in a developer monobath of the following composition:

|                                 |      |     |
|---------------------------------|------|-----|
| Water                           | 800  | ml. |
| Sodium hexametaphosphate        | 2.0  | g.  |
| 2-methyl-4-diethylamino aniline | 12.0 | g.  |
| Sodium sulfite                  | 50.0 | g.  |
| Chlorohydroquinone              | 6.0  | g.  |
| Sodium carbonate (anhydrous)    | 40.0 | g.  |
| Potassium bromide               | 2.0  | g.  |
| Water to                        | 1000 | ml. |

The film was then treated according to the procedure of Example 1. The following densitometric results were obtained:

|                | Dmin | Dmax |
|----------------|------|------|
| to Blue light  | 0.30 | 3.30 |
| to Green light | 0.52 | 3.10 |
| to Red light   | 0.60 | 3.76 |

#### EXAMPLE 4

A silver halide photographic element similar to that employed in Example 1 was exposed to light through a grey wedge and then developed for 5 minutes at 70°F. in total darkness in a developer monobath of the following composition:

|                                 |      |     |
|---------------------------------|------|-----|
| Water                           | 800  | ml. |
| Sodium hexametaphosphate        | 2.0  | g.  |
| 2-methyl-4-diethylamino aniline | 12.0 | g.  |
| Sodium sulfite                  | 50.0 | g.  |
| Methyl-para-aminophenol sulfate | 6.0  | g.  |
| Sodium carbonate (anhydrous)    | 40.0 | g.  |
| Potassium bromide               | 2.0  | g.  |
| Water to                        | 1000 | ml. |

The film was then processed in accordance with Example 1. The following densitometric properties were obtained:

|                | Dmin | Dmax |
|----------------|------|------|
| to Blue light  | 0.50 | 3.42 |
| to Green light | 1.20 | 2.92 |
| to Red light   | 0.80 | 3.70 |

#### EXAMPLE 5

Example 1 was duplicated exactly with similar photographic material except that, in the monobath, 9.0 g. of p-hydroxyphenylglycin was substituted for hydroquinone. The following densitometric properties were obtained:

|                | Dmin | Dmax |
|----------------|------|------|
| to Blue light  | 0.30 | 2.88 |
| to Green light | 0.86 | 3.72 |
| to Red light   | 0.70 | 3.52 |

#### EXAMPLE 6

A photographic silver halide color reversal film similar to that employed in Example 1 was exposed through a grey wedge in a sensitometer and was then developed for 3 minutes at 70°F. in total darkness with agitation in a developer monobath of the following composition:

|                                                             |      |     |
|-------------------------------------------------------------|------|-----|
| Water                                                       | 800  | ml. |
| Sodium hexametaphosphate                                    | 2.0  | g.  |
| p-(N-ethyl-N-β-hydroxyethyl)-aminoaniline (color developer) | 18.0 | g.  |
| Potassium sulfite                                           | 48.0 | g.  |
| Hydroquinone                                                | 7.5  | g.  |
| 1-phenyl-3-pyrazolidinone                                   | 0.30 | g.  |
| Potassium bromide                                           | 2.0  | g.  |
| Sodium carbonate (anhydrous)                                | 30.0 | g.  |
| Sodium hydroxide                                            | 4.0  | g.  |
| Water to                                                    | 1000 | ml. |

10 The film was thereafter placed in a second bath of:

|                                                      |     |     |
|------------------------------------------------------|-----|-----|
| Water                                                | 800 | ml. |
| Na <sub>2</sub> PO <sub>4</sub> ·12 H <sub>2</sub> O | 4.0 | g.  |
| Sodium hydroxide                                     | 4.0 | g.  |

and was re-exposed to room light illumination therein for 3 minutes. The film was then washed, bleached, fixed, washed and dried according to the procedure of

20 Example 1. The following densitometric properties were obtained:

|                | Dmin | Dmax |
|----------------|------|------|
| to Blue light  | 0.35 | 4.80 |
| to Green light | 0.16 | 2.24 |
| to Red light   | 0.12 | 3.50 |

#### EXAMPLE 7

A color reversal silver halide photographic film similar to that of Example 6 was exposed to a light image and then developed for 4 minutes at 70°F. in total darkness in a developer monobath of the following composition:

|                                                         |      |     |
|---------------------------------------------------------|------|-----|
| Water                                                   | 800  | ml. |
| Sodium hexametaphosphate                                | 2.0  | g.  |
| Potassium sulfite                                       | 48.0 | g.  |
| Benzyl alcohol                                          | 3.5  | g.  |
| Ethylene glycol                                         | 4.5  | g.  |
| p-(N-ethyl-N-β-hydroxyethyl)-aminoaniline, sulfate salt | 18.0 | g.  |
| Hydroquinone                                            | 7.5  | g.  |
| 1-phenyl-3-pyrazolidinone                               | 0.30 | g.  |
| Sodium thiocyanate                                      | 0.5  | g.  |
| Potassium bromide                                       | 2.0  | g.  |
| Potassium iodide                                        | 0.01 | g.  |
| Sodium carbonate (anhydrous)                            | 30.0 | g.  |
| Sodium hydroxide                                        | 4.0  | g.  |
| Water to                                                | 1000 | ml. |

50 The film was then washed for 2 seconds with water and then re-exposed to light. Thereafter the film was placed in a bath containing a mixture of 4.0 g. per liter of trisodium phosphate dodecahydrate and 4.0 g. per liter of sodium hydroxide for 3 minutes. Thereafter, the film was treated consecutively in a short stop solution (1 minute), a bleach bath (2.5 minutes), a fixing bath (2 minutes) and was then washed for 1 minute, placed in a stabilizing (formaldehyde) bath for 1 minute, and 55 dried. Ingredients of the short stop, bleach and fix baths are as follows:

|                        |      |     |
|------------------------|------|-----|
| 65 Short Stop Solution |      |     |
| Glacial acetic acid    | 12.0 | ml. |
| Sodium acetate         | 6.3  | g.  |
| Water to               | 1000 | ml. |

## Bleach Bath

|                             |       |     |
|-----------------------------|-------|-----|
| Water                       | 800   | ml. |
| Potassium ferricyanide      | 112.0 | g.  |
| Potassium bromide           | 24.0  | g.  |
| Disodium hydrogen phosphate | 12.0  | g.  |
| Sodium thiocyanate          | 12.5  | g.  |
| Sodium dihydrogen phosphate | 12.5  | g.  |
| Water to                    | 1000  | ml. |

## Fixing Bath

|                                                |       |     |
|------------------------------------------------|-------|-----|
| Water                                          | 800   | ml. |
| Ammonium thiosulfate<br>(60% aqueous solution) | 120.0 | g.  |
| Sodium metabisulfite                           | 20.0  | g.  |
| Water to                                       | 1000  | ml. |

The following densitometric properties were obtained:

|                | Dmin | Dmax |
|----------------|------|------|
| to Blue light  | 0.19 | 5.20 |
| to Green light | 0.11 | 3.21 |
| to Red light   | 0.08 | 3.58 |

## EXAMPLE 8

Example 1 was duplicated exactly except that the amount of hydroquinone was reduced from 6 grams to 2 grams in the monobath solution. The following densitometric properties were obtained:

|                | Dmin | Dmax |
|----------------|------|------|
| to Blue light  | 0.96 | 4.70 |
| to Green light | 0.86 | 3.36 |
| to Red light   | 0.62 | 2.22 |

## EXAMPLE 9

A photographic silver halide black and white material (coupler-free) was exposed through a grey wedge in a sensitometer and was then developed for 2 minutes at 70°F. in total darkness in a developer monobath resulting from combining 300 ml. of the following solution A with the following solution B:

## Solution A

|                                 |      |     |
|---------------------------------|------|-----|
| Water                           | 800  | ml. |
| Sodium hexametaphosphate        | 2.0  | g.  |
| 2-methyl-4-diethylamino aniline | 12   | g.  |
| Sodium sulfite                  | 50   | g.  |
| Hydroquinone                    | 6.0  | g.  |
| Sodium carbonate (anhydrous)    | 40.0 | g.  |
| Potassium bromide               | 2.0  | g.  |
| Water to                        | 1000 | ml. |

## Solution B

|                                                                            |     |     |
|----------------------------------------------------------------------------|-----|-----|
| Water                                                                      | 50  | ml. |
| Sodium carbonate                                                           | 2.0 | g.  |
| N-(1-hydroxy-2-naphthoyl)-N-hexadecyl-3,5-dicarboxy aniline (cyan coupler) | 3.0 | g.  |

The film was then placed in an aqueous solution containing 40 g. per liter of sodium carbonate, and exposed to room light illumination therein for 3 minutes. The film was then washed, bleached, fixed, washed and dried in accordance with Example 1. A positive color monochrome image having the following densitometric properties was obtained:

Dmin Dmax

|              |      |      |
|--------------|------|------|
| to Red light | 0.58 | 0.72 |
|--------------|------|------|

5

## EXAMPLE 10

A silver halide color photographic element of the type described in Example 1 was exposed to light through a grey wedge and then developed for 3 minutes at 70°F. in total darkness in the developing solution monobath of Example 1. The film was then immersed for 3 minutes in a second bath, maintaining total darkness conditions. The second bath consisted of:

15

|                              |      |             |
|------------------------------|------|-------------|
| Water                        | 1000 | ml. (total) |
| Sodium carbonate (anhydrous) | 40   | g.          |
| Potassium borohydride        | 0.05 | g.          |

20 The film thereafter was fixed in the fixing solution of Example 1 for 2 minutes, also in total darkness, and was then further washed, bleached, fixed, washed and dried in accordance with Example 1. The film, now bearing a positive color image, exhibited the following densitometric characteristics:

|                  | Dmin | Dmax |
|------------------|------|------|
| 30 to Blue light | 0.21 | 2.27 |
| to Green light   | 0.42 | 3.10 |
| to Red light     | 0.78 | 3.38 |

## EXAMPLE 11

35 A color reversal silver halide photographic material similar to that of Example 6 was exposed to light through a grey wedge and then developed for 4 minutes at 70°F. in total darkness in a developer solution of the following composition:

40

|                                                         |      |     |
|---------------------------------------------------------|------|-----|
| Water                                                   | 800  | ml. |
| Sodium hexametaphosphate                                | 2.0  | g.  |
| p-(N-ethyl-N-β-hydroxyethyl)-aminoaniline, sulfate salt | 18.0 | g.  |
| Potassium sulfite                                       | 20.0 | g.  |
| Hydroquinone Monocarboxylic acid hydrazide              | 11.5 | g.  |
| Potassium bromide                                       | 2.0  | g.  |
| Sodium carbonate (anhydrous)                            | 30.0 | g.  |
| Sodium hydroxide                                        | 4.0  | g.  |
| Water to                                                | 1000 | ml. |

50

The film was thereafter treated in accordance with Example 6. The following densitometric properties were obtained:

55

|                | Dmin | Dmax |
|----------------|------|------|
| to Blue light  | 0.70 | 2.20 |
| to Green light | 0.44 | 4.10 |
| to Red light   | 0.60 | 4.20 |

60

## EXAMPLE 12

65 A color reversal silver halide photographic element similar to that of Example 6 was exposed to light through a grey wedge and then developed for 3 minutes at 70°F. in total darkness in a developer monobath of the following composition:

|                                               |      |     |
|-----------------------------------------------|------|-----|
| Water                                         | 800  | ml. |
| Sodium hexametaphosphate                      | 2.0  | g.  |
| p-(N-ethyl-N-β-hydroxyethyl)-<br>aminoaniline | 18.0 | g.  |
| Ascorbic acid                                 | 44.0 | g.  |
| Hydroquinone                                  | 7.5  | g.  |
| 1-phenyl-3-pyrazolidinone                     | 0.30 | g.  |
| Potassium bromide                             | 2.0  | g.  |
| Sodium carbonate (anhydrous)                  | 30.0 | g.  |
| Sodium hydroxide                              | 4.0  | g.  |
| Water to                                      | 1000 | ml. |

The film was thereafter immersed in a second bath of 10 the following composition and re-exposed therein to room light illumination for 3 minutes:

|                                |      |     |
|--------------------------------|------|-----|
| Water                          | 800  | ml. |
| Sodium phosphate dodecahydrate | 4.0  | g.  |
| Sodium hydroxide               | 4.0  | g.  |
| Water to                       | 1000 | ml. |

The film was thereafter washed, bleached, fixed, washed and dried according to Example 1. The following densitometric properties were obtained:

|                | D <sub>min</sub> | D <sub>max</sub> |    |
|----------------|------------------|------------------|----|
| to Blue light  | 0.55             | 2.30             | 25 |
| to Green light | 0.42             | 1.46             |    |
| to Red light   | 0.52             | 2.60             |    |

### EXAMPLE 13

A kit for preparing a monobath of the invention was formulated as follows into two packages:

| <u>Package A</u>                              |      |    |  |
|-----------------------------------------------|------|----|--|
| Sodium hexametaphosphate                      | 2.0  | g. |  |
| p-(N-ethyl-N-β-hydroxyethyl)-<br>aminoaniline | 18.0 | g. |  |
| Potassium sulfite                             | 48.0 | g. |  |
| Hydroquinone                                  | 7.5  | g. |  |
| 1-phenyl-3-pyrazolidinone                     | 0.30 | g. |  |

  

| <u>Package B</u>  |      |    |  |
|-------------------|------|----|--|
| Sodium carbonate  | 30.0 | g. |  |
| Sodium hydroxide  | 4.0  | g. |  |
| Potassium bromide | 2.0  | g. |  |

In use, the contents of package A are dissolved in 700 ml. of water, and the contents of package B are dissolved in 200 ml. of water. The resulting solutions are then combined and diluted to 1000 ml. to provide a working monobath solution of the invention.

### EXAMPLE 14

This example illustrates the inhibiting mechanism whereby oxidation of the color developer is prevented by blocking the developer.

#### Developer Composition

|                   |      |     |
|-------------------|------|-----|
| Calgon*           | 2.0  | g.  |
| CD-2**            | 12.0 | g.  |
| Sodium Sulfite    | 50.0 | g.  |
| Amidol            | 10.0 | g.  |
| Potassium Bromide | 2.0  | g.  |
| Water dilute to   | 1000 | ml. |

\*Na hexametaphosphate

\*\*2-amino-5-diethylaminotoluene monohydrochloride

Ferrania Mark III cine positive release film was used to reduce this invention to practice. This material can

be processed reversibly to yield color positive transparencies of good quality and may be considered representative of any commercially available negative acting color silver halide material or any color silver halide 5 material designed for conventional reversal processing. The color couplers in the material are resin dispersed, although the invention is not limited to such a particular composition. The construction of the tripack is adequately described in the prior art.

A test strip of this material was exposed on an EK101 sensitometer for 2 seconds before a logarithmic step wedge. This strip was processed in the development formulation described in this example for 4 minutes at 70°F in total darkness. After this development period, 10 the test strip was removed from the development bath and placed in a bath containing 40.0 g/l of Na<sub>2</sub>CO<sub>3</sub> for 3 minutes while being exposed to room light illumination. During this time, dye formation was noted to take place. After this period, the test strip was subjected to conventional ferricyanide bleach, wash, stop-fix, wash and stabilization steps; any step of which does not impose any limitations on this invention. This treatment resulted in the production of a color positive image of 20 the following densitometric characteristics:

|                  | Red  | Blue | Green |
|------------------|------|------|-------|
| D <sub>max</sub> | 3.20 | 2.70 | 2.72  |
| D <sub>min</sub> | 0.32 | 0.08 | 0.70  |
| Gamma            | 4.3  | 2.6  | 3.7   |

If a water wash bath is used for the re-exposure step, no dye density is produced in the test strip, indicating that the pH rise of this example is necessary to activate the 35 color developer.

Although the sulfite concentration in this example is such as could be sufficient to act as an inhibitor by forming a reaction product with oxidized color developing agent, the pH of this bath is such that there can 40 be no oxidation of the color developer. The sulfite is present only as a stabilizer and does not here inhibit coupling of oxidized color developer, as there is none until the pH is raised.

What is claimed is:

1. A bath for photographic positive color development of silver halide photographic elements, said bath comprising, in aqueous solution at a pH of from 8.5 to 14:
  - 50 A. at least 0.02 moles/liter of photographic color developing agent capable, upon oxidation thereof, of reacting with a photographic coupler to form a dye; said color developing agent having a polarographic half-wave potential at pH 11.0 from about -159 to about -305 millivolts;
  - B. at least one black and white developing agent having a polarographic half-wave potential at pH 10.0 of from about -10 millivolts to about -187 millivolts; and
  - C. water-soluble, dye-formation inhibitor in a concentration of at least about 0.10 moles/liter which is present in sufficient quantity so that substantially all dye formation of a silver halide photographic element is restrained in said bath after said element has been exposed to light, the mole ratio of inhibitor to color developer being at least about 0.97.
2. The bath according to claim 1 wherein said dye-formation inhibitor is sulfite.

3. The bath according to claim 1 wherein the pH thereof is from about 10 to about 11.
4. The bath according to claim 1 wherein the dye-formation inhibitor is capable of forming a reaction product with the oxidation product of said color developing agent. 5
5. The bath according to claim 1 wherein the dye-formation inhibitor is capable of preventing the color developing agent from being oxidized.
6. The developer bath according to claim 1 wherein said color developing agent represents from about 40 to about 95 mole percent of the total developer content of said bath. 10

7. The developer bath of claim 1 wherein said at least one black and white photographic developing agent is hydroquinone. 15

8. The developer bath according to claim 1 which additionally includes a color coupler compound.

9. The developer bath according to claim 1 wherein said at least one color developing agent has a polarographic half-wave potential at pH 11.0 of from about -159 millivolts to about -305 millivolts. 20

10. The bath of claim 1 wherein the dye formation inhibitor is selected from the group consisting of sulfite, ascorbic acid, citrazinic acid, 4-hydroxy-3-butanone and hydroquinone monocarboxylic acid hydrazides. 25

11. The bath of claim 1 wherein the pH is at least 10.0.

12. A color developer bath for positive color development of silver halide photographic elements, said bath comprising, in aqueous solution of pH 8.5-14,

A. at least 0.02 moles/liter of primary aromatic amine photographic color developing agent capable, upon oxidation thereof, of reacting with a photographic color coupler to form a dye, said color developing agent having a polarographic half-wave potential at pH 11.0 of from about -159 to about -305 millivolts;

B. at least one black and white developing agent having a polarographic half-wave potential at pH 10.0 of from about -10 millivolts to about -187 millivolts; and

C. from about 0.10 to about 0.48 moles/liter of inhibitor which is present in sufficient quantity so that substantially all dye formation of a silver halide photographic element is restrained in said bath after said element has been exposed to light, and which forms a reaction product with oxidized said color developing agent, the mole ratio of inhibitor to color developer being at least about 0.97. 45

13. The developer bath according to claim 12 wherein said inhibitor is sulfite.

14. The developer according to claim 12 wherein said black and white photographic developer includes hydroquinone and 1-phenyl-3-pyrazolidinone. 55

15. A photographic color reversal development process which comprises

A. treating a color photographic element having a hydrophilic colloid silver halide layer bearing a latent image with an aqueous bath solution which includes at least 0.02 moles/liter of photographic color developing agent capable, upon oxidation, of reacting with a photographic color coupler to form a dye, black and white photographic developer including at least one black and white developing agent having a polarographic half-wave potential at pH 10.0 of from about -10 millivolts to about

-187 millivolts, and water-soluble dye-formation inhibitor in a concentration of at least 0.10 moles/liter, said concentration being sufficient so that substantially all dye formation of a silver halide photographic element is restrained in said bath after said element has been exposed to the light, the mole ratio of inhibitor to color developer being at least about 0.97, thereby to imbibe said silver halide layer with said bath solution and to develop solely a negative black and white image therein;

B. thereafter fogging said silver halide layer so as to render said layer developable in non-imaged areas; C. without intermediate removal of said imbibed bath solution, treating said layer to reduce the inhibiting effect of said dye formation inhibitor; and D. allowing development therein of a positive color image in the presence of a color coupler.

16. The process according to claim 15 wherein said color coupler is originally in the photographic element.

17. The process according to claim 15 wherein at least some of the presence of color coupler is supplied by a bath.

18. The process according to claim 15 wherein the fogging and reduction of inhibiting effect is performed in the same bath.

19. The process according to claim 15 wherein said element is washed with an inhibitor-dissolving aqueous solution after said fogging step.

20. The process according to claim 15 wherein said fogging step comprises exposing said film bearing said black and white silver image to light.

21. The process according to claim 15 wherein said fogging step comprises treating said film bearing said black and white silver image with a fogging agent.

22. The process according to claim 15 wherein the pH of the bath is about 8.5-14.

23. The process according to claim 15 wherein any baths of the group selected from stop baths, bleach baths, fix baths, bleach/fix baths, wash baths, stabilizing baths, or hardening baths are also used.

24. A photographic color reversal development process which comprises

A. treating a photographic element having a hydrophilic colloid silver halide layer bearing a latent image with an aqueous alkaline bath which includes at least 0.02 moles/liter of primary aromatic amine color developing agent capable, upon oxidation thereof, of reacting with a photographic coupler to form a dye, said color developing agent having a polarographic half-wave potential at pH 11.0 of from about -159 to about -305 millivolts, black and white photographic developer which includes hydroquinone, and from 0.10 to 0.48 moles/liter of inhibitor in a concentration sufficient so that substantially all dye formation of a silver halide photographic element is restrained in said bath after said element has been exposed to light, the mole ratio of inhibitor to color developer being at least about 0.97, thereby to imbibe said bath into said silver halide layer and to develop solely a negative black and white silver image therein;

B. thereafter fogging said silver halide layer by exposure thereof to light; and

C. without intermediate removal of imbibed bath, washing said layer with an inhibitor-dissolving aqueous alkaline solution until a positive color image has been developed therein.

25. The process according to claim 24 wherein said inhibitor is sulfite.
26. A color developer bath for photographic positive color development of silver halide photographic elements, said bath comprising, in aqueous solution of pH 8.5-14,
- A. at least 0.02 moles/liter of a photographic color developing agent capable of reacting with a photographic color coupler to form a dye, said color developing agent having a polarographic half-wave potential at pH 11.0 of from about -159 to about -305 millivolts;
  - B. a black and white photographic developer including at least one black and white developing agent having a polarographic half-wave potential at pH 10.0 of from about -10 millivolts to about -187 millivolts; and
  - C. a water-soluble, dye-formation inhibitor in a concentration of at least about 0.10 moles/liter which is capable of reacting with the oxidation product of said color developing agent to form a stable, soluble complex and which is present in sufficient quantity so that substantially all dye formation of a silver halide photographic element is restrained in said bath after exposure of said element to light, the mole ratio of inhibitor to color developer being at least about 0.97.
27. A photographic color reversal development process which comprises
- A. treating a photographic element having a hydrophilic colloid silver halide layer bearing a latent image with an aqueous alkaline bath which includes at least 0.02 moles/liter of photographic color developing agent capable, upon oxidation of reacting with a photographic color coupler to form a dye, black and white photographic developer including at least one black and white developing agent having a polarographic half-wave potential at pH 10.0 of from about -10 millivolts to about -187 millivolts, and water-soluble dye-formation inhibitor in a concentration sufficient so that substantially all dye formation of a silver halide photographic element is restrained in said bath after said element has been exposed to light, and of at least about 0.10 moles/liter, the mole ratio of inhibitor to color developer being at least about 0.97, thereby to imbibe said silver halide layer with said bath and to develop solely a negative black and white silver image therein;
  - B. thereafter fogging said silver halide layer so as to render said layer developable in non-imaged areas; and
  - C. without intermediate removal of said imbibed

- bath, treating said layer to reduce the inhibiting effect of said dye formation inhibitor, thereby to cause development therein of a positive color image.
28. A bath for photographic positive color development of silver halide photographic elements said bath comprising in aqueous solution at a pH of from 8.5-14;
- A. at least 0.02 moles/liter of photographic color developing agent capable, upon oxidation thereof, of reacting with a photographic coupler to form a dye, said color developing agent having a polarographic half-wave potential at pH 11.0 of from about -159 to about -305 millivolts,
  - B. at least one black-and-white developing agent having a polarographic half-wave potential at pH 10.0 of from about -10 millivolts to about -187 millivolts, and
  - C. water-soluble, dye-formation inhibitor in a concentration which is sufficient so that substantially all dye formation of a silver halide photographic element is restrained in said bath after said element has been exposed to light, the mole ratio of inhibitor to color developer being at least about 0.97.
29. The bath of claim 28 wherein the dye formation inhibitor is selected from the group consisting of sulfite, ascorbic acid, citrazinic acid, 4-hydroxy-3-butanone and hydroquinone monocarboxylic acid hydrazides.
30. A bath for photographic positive color development of silver halide photographic elements, said bath comprising in aqueous solution at a pH of from 8.5-14;
- A. at least 0.02 moles/liter of photographic color developing agent capable, upon oxidation thereof, of reacting with a photographic coupler to form a dye, said color developing agent having a polarographic half-wave potential at pH 11.0 of from about -159 to about -305 millivolts,
  - B. at least one black and white developing agent having a polarographic half-wave potential at pH 10.0 greater than that of phenidone to -10 millivolts, and
  - C. water-soluble, dye-formation inhibitor in a sufficient concentration so that substantially all dye formation of a silver halide photographic element is restrained in said bath after said element has been exposed to light, the mole ratio of inhibitor to color developer being at least about 0.97.
31. The photographic developer bath of claim 30 in which dye formation inhibitor is present in a concentration of at least about 0.10 moles/liter.
32. The bath of claim 30 wherein the dye formation inhibitor is selected from the group consisting of sulfite, ascorbic acid, citrazinic acid 4-hydroxy-3-butanone, and monocarboxylic acid hydrazides.